

W. E. KIMBER,  
MANUFACTURE OF TOOLS FOR TURNING, BORING, AND SIMILAR PURPOSES,  
APPLICATION FILED NOV. 13, 1918.

1,859,459.

Patented Nov. 16, 1920.

Fig. 1.



Fig. 2.



Fig. 4. 1



Inventor  
Walter Edward Kimber  
By Frank Chase Jones  
Attorney.

# UNITED STATES PATENT OFFICE.

WALTER EDWARD KIMBER, OF LONDON, ENGLAND.

MANUFACTURE OF TOOLS FOR TURNING, BORING, AND SIMILAR PURPOSES.

1,359,459.

Specification of Letters Patent. Patented Nov. 16, 1920.

Application filed November 13, 1918. Serial No. 262,847.

To all whom it may concern:

Be it known that I, WALTER EDWARD KIMBER, a subject of the King of Great Britain, residing at 87 Saint Augustine's Road, Cam-  
5 den Square, London, N. W. 1, England, have invented new and useful Improvements in and Connected with the Manufacture of Tools for Turning, Boring, and Similar Purposes, of which the following is a speci-  
10 fication.

The invention relates to the method of producing a composite bar for the production of tools for turning, planing, boring and similar purposes and comprising a shank 15 or stem of mild or carbon steel with a portion of high speed steel attached thereto in the position where the operative or acting edge of such tool is desired to be formed, and the essential or characteristic feature 20 is the attachment of the two portions by a fused joint or connection through their point of contact, and which is effected with the total exclusion of air and while the high speed steel is in the necessary molten condition to insure the fusion of the portion of 25 the carbon tool steel with which it is brought into contact.

A comparatively small portion of the shank only is required to receive the high speed steel and it is this portion which is introduced into a pocket of refractory material which can be handled and manipulated so as to insure the required conditions being fulfilled, and which is secured by the 30 previous insertion of the shank of carbon steel into the refractory pocket and the immersion of same into a bath of molten high speed steel to allow the latter to enter the pocket through an opening therein when it is 35 plunged or immersed below the surface. The shank is protected against total fusion during immersion in the molten high speed steel by the refractory pocket and said molten metal is permitted to come in contact 40 with a small edge or area only of the shank. The molten high speed steel is of so high a temperature (about 1800° C.) that the immersion therein of an unprotected shank of 45 mild steel would cause the immediate fusion 50 and disappearance of said shank into the mass of molten metal.

The method is not a casting process, but essentially a fusing process by immersion.

By the immersion of the whole pocket in 55 molten metal all access of air is entirely prevented, and consequent oxidation rendered

impossible, and the placing of the pocket with the contained portion of shank together under the steel, the molten metal outside the pocket allows the molten metal inside the 60 pocket to remain in a molten condition for as long as is required to effect perfect fusion, and as a fact if allowed to remain for too long a period the whole thing—viz. the shank inclusive would be reduced to a molten 65 condition.

The exposure of a small portion of high speed steel in a molten condition to the atmosphere entirely deteriorates same by oxidation so as to render it useless.

The immersion of the shank when in the pocket into molten steel and its removal in such pocket therefrom with the small portion of high speed steel attached thereto entirely prevents all possibility of access of air 70 to the portion during the whole operation of its attachment.

In the accompanying drawing illustrating the manner of carrying my invention into effect—

Figure 1 is a vertical section through the pocket of highly refractory material employed to receive the portion of the body or stem to which the high speed steel is to be applied.

Fig. 2 a plan view thereof or partly in section.

Fig. 3 an elevation of the lower end of the body or stem after removal from the pocket and as indicated by the shade or section lines 90 with the applied portion of high speed steel shaped to the desired form.

Fig. 4 is a vertical section of the lower portion of the pocket shown in Fig. 1 provided with an opening near the bottom 95 thereof, through which molten steel may enter.

For the purpose of this invention a length of mild steel preferably of rectangular section and of a suitable length and shape is 100 employed to approximately constitute the body or stem 1 but with a portion 2 omitted or removed where the cutting or operative edge of the tool is required to be formed, and which extends back along such body or 105 stem a sufficient distance to afford an effective bearing surface for the welded joint with the portion of the high speed steel 3 it is intended to receive.

The body or stem 1 so shaped is introduced into a pocket 4 of highly refractory material such as Sheffield clay as used for

steel melting crucibles, and the interior of which is shaped so that when the stem 1 bears on the bottom thereof with the enlarged portion inserted within the mouth of 5 the pocket, a clear space 5 will be left opposite the removed portion of the stem.

The opening in the pocket 4 is at the bottom recessed or reduced at 6 to receive the 10 end of the reduced portion of the stem 1 which is inserted therein, so as to hold the stem in position within the pocket with the clear space 5 of uniform depth throughout its length on that side to which the high speed steel 3 is to be applied.

15 An opening 7 through the wall of the pocket 4 opposite such space 5 communicates with the interior at a point near the top thereof, and such wall is, as shown, advantageously made thinner than the remaining walls or sides of the pocket.

20 After the stem 1 has been introduced a wedge 8 of refractory material is inserted in the mouth of the pocket 4 to fix same therein and close the clearance which exists between it and the wall on one side, while the other sides may if necessary be sealed with refractory clay.

25 The pocket 4 with the stem 1 inserted therein is preheated to a bright red heat and 30 then plunged into a pot of molten high speed steel (to the level indicated at 9 in Fig. 1) until the hole 7 near the top of the pocket is submerged, which allows such high speed steel to pass to the interior and fill 35 the space 5 left where the removed portion 2 of the stem 1 is situated. The pocket 4 is allowed to remain submerged for a sufficient length of time (about a minute or two) to enable the entering high speed steel 40 3 to act upon the surface of the stem 1 to which it is required to unite to bring same to and maintain it at a fusing heat, the decreased thickness of the wall through which the molten steel enters in comparison to that 45 of the other walls of the pocket, assisting this action by the greater radiation of heat through same from the outer molten steel in the pot in which the pocket is submerged.

An opening 10 indicated in dotted lines 50 in Fig. 1, may also be provided near the bottom of the pocket 4 so that the molten steel may pass to the space in the interior at both bottom and top, and to prevent the metal running back as the pocket is withdrawn 55 such bottom opening 10 might be first closed by refractory clay forced down on the end of a rod, before the removal of the pocket from the pot is effected. This opening 10 may be omitted.

60 After the necessary immersion the pocket 4 is withdrawn from the pot with the stem 1 it contains and the high speed steel which has entered same, and is immediately plunged into or covered with refractory material, such as sand, to prevent the possibil-

ity of access of air, and allowed to remain until sufficiently cool to permit of the removal of the pocket, which may be broken off leaving the stem 1 with the portion of high speed steel 3 securely attached thereto 70 by fusion at the position 2 reserved for its reception.

The inclosing of the portion of the stem 1 which is to receive the high speed steel within the pocket 4 during the fusing or 75 joining of such high speed steel thereto, by excluding all access of air insures the formation of an efficient joint, all risk of oxidation of the high speed steel being effectually prevented.

80 The space provided in the pocket 4 is preferably such as will insure an excess of attached high speed steel 3 on the stem 1 to that required to fill the space 2 reserved therefor, which excess will as illustrated in 85 Fig. 3 allow for the forging or shaping necessary of the combined or composite bar of mild steel and high speed steel to the required form to present the necessary cutting or operative surface at the desired point.

85 The high speed steel might be melted in the pocket 4 itself and the stem 1 after pre-heating be plunged into the molten metal and the whole allowed to remain until the 90 desired fusion is effected, when the pocket 4 with the stem 1 therein would be removed from the furnace in which it had been heated, and treated in the same manner as above described.

95 100 What I claim as my invention, and desire to secure by Letters Patent, is:—

1. The method of producing a composite bar of mild and high speed steel for formation of tools for turning and like purposes which consists in fixing in a refractory apertured pocket a stem of mild steel with a portion of its surface spaced from the wall of said pocket, immersing said pocket and contained stem in a molten bath of high speed steel and subjecting the said protected stem bodily to the indirect heat of said bath and along the spaced portion thereof simultaneously to direct contact of the inflow of molten bath high speed steel until said 115 spaced surface is brought to a fusing heat and united with the metal of said inflow, and then withdrawing said pocket and contents from said bath.

120 125 130 2. The method of producing a composite bar of mild and high speed steel for formation of tools for turning and like purposes which consists in fixing in a refractory apertured pocket a stem of mild steel with a portion of its surface spaced from the wall of said pocket, subjecting said stem while in said pocket to a red heat, immersing said pocket and contained stem in a molten bath of high speed steel and subjecting the said protected stem bodily to the indirect heat of

said bath and along the spaced portion thereof simultaneously to direct contact of the inflow of molten bath high speed steel until said spaced surface is brought to a 5 fusing heat and united with the metal of said inflow, and then withdrawing said pocket and contents from said bath.

3. The method of producing a composite bar of mild and high speed steel for 10 formation of tools for turning and like purposes which consists in forming a stem of mild steel or carbon tool steel with a recess through a portion of its length, fixing in a refractory apertured pocket said stem of 15 mild steel with the recessed portion of its surface spaced from the wall of said pocket, immersing said pocket and contained stem

in a molten bath of high speed steel and subjecting the said protected stem bodily to the indirect heat of said bath and along the 20 spaced portion thereof simultaneously to direct contact of the inflow of molten bath high speed steel until said spaced surface is brought to a fusing heat and united with the metal of said inflow, and then withdrawing 25 said pocket and contents from said bath.

In testimony whereof I have signed my name to this specification in the presence of two subscribing witnesses.

WALTER EDWARD KIMBER.

Witnesses:

LAWRENCE G. LEE,  
WILLIAM JAS. FERRY.